

# UNITED STATES PATENT OFFICE.

CLIFFORD D. HOLLEY, OF DETROIT, MICHIGAN, ASSIGNOR TO ACME WHITE LEAD AND COLOR WORKS, OF DETROIT, MICHIGAN, A CORPORATION OF MICHIGAN.

## PROCESS OF OXIDIZING LEAD.

1,116,702.

Specification of Letters Patent. Patented Nov. 10, 1914.

No Drawing.

Application filed February 11, 1911. Serial No. 608,105.

To all whom it may concern:

Be it known that I, CLIFFORD D. HOLLEY, a citizen of the United States, residing at Detroit, in the county of Wayne and State of Michigan, have invented certain new and useful Improvements in Processes of Oxidizing Lead, of which the following is a specification.

This invention relates to processes of oxidizing lead; and it comprises a method of oxidizing metallic lead wherein finely-divided lead is oxidized by air in the presence of a solution containing the nitrate of an alkali metal as a catalytic or facilitating agent, such nitrate being ordinarily subsequently regained as an alkali nitrite; such solution being advantageously a waste liquor derived from the manufacture of lead chromate and containing an alkali nitrate, such as sodium nitrate, as well as, usually, free nitric acid; all as more fully hereinafter set forth and as claimed.

When submerged in or wet with water, bright surfaces of metallic lead are oxidized by air, if air has access to the liquid, with the production of a hydrated oxid of lead of basic and reactive properties. With water alone the reaction never goes very far, neither is it very rapid, even in "attrition" processes where the lead oxid formed is kept scoured off by attrition. With water containing saline or other ionizable substances, such as acids, and particularly where these acids, as is the case with nitric and acetic acids, form soluble lead salts, the action is facilitated, partly, probably, at first by removal of the oxid from the affected surfaces in the case of the acids and partly, probably, for more obscure reasons connected with the presence of ions. Both acetic and nitric acids have been proposed for use in such processes. The former is, directly or indirectly, the corroding agent in the well known Dutch process, which, while yielding a high grade pigment, is relatively very slow and expensive. The use of nitric acid in proposed processes of making lead oxid has, as a rule, not been successful in practice. In my copending application Serial No. 588,973, filed October 25, 1910, I have, however, disclosed a commercially practicable method of making oxids of lead in which nitric acid is employed. In the aforesaid application I have also disclosed, but have not claimed specifically, a modified

process in which nitrates such as sodium nitrate and the like, either alone or in connection with nitric acid, may take the place of nitric acid *per se*. The present application is in part, therefore, a continuation of my prior application aforesaid. Where nitric acid alone is employed it is apt to undergo a far-going reduction, first forming lead nitrates and then nitrites with, ultimately, formation of neutral nitrogen oxids and ammonia. Acids of course do not long remain as such in the presence of the lead undergoing oxidation, but become converted into lead salts by reaction with the lead oxid produced.

I have discovered that, for some purposes a much better facilitating or catalytic agent is to be found in solutions of the nitrates of the alkalis, such as nitrate of sodium or nitrate of potassium, the former being the better. Nitrates of alkaline earths, such as nitrate of calcium, barium, strontium and magnesium are less suitable and do not yield commercially valuable by-products. Unlike the nitrate of lead, the alkali nitrates do not undergo a far-reaching reduction but are converted into nitrites from which in the course of the operation nitrates are probably regenerated by the action of the air; these nitrates thus acting as carrier agents. Whatever may be the chemical mechanism of the reactions involved, I have found that a solution of an alkali nitrate, and particularly a solution of sodium nitrate, acts as an energetic oxidizing agent in the corrosion of lead in the presence of water and air, quickening the operation very materially and giving a desirable type of hydrated basic and reactive oxid of lead from which white lead, massicot, litharge, minium and other pigmentary lead products of good quality may be made. As is well known, the pigmentary value of oxidized lead products depends very much on their molecular constitution; it being practically impossible, for example, to make a good red lead, or, in fact, commercially, any red lead, from some forms of lead oxid, as for example, from fused litharge. The hydrated oxid made under the present invention is reactive and molecularly fine and, with proper methods of treatment, carries its reactivity and fineness of constitution throughout in conversion into other and pigmentary lead products; giving, for example, a fine-grained

white lead of good covering power, a fine high grade minium or red lead of unusual volume for its weight, etc.

After the oxidation of lead in the presence of a solution of an alkali nitrate, the latter is converted into and remains in such solution as an alkali nitrite; sodium nitrate, for example, becoming sodium nitrite, a commercially valuable product useful for many purposes, as in the dye and color industries. This nitrite may be regained, as by evaporation of the residual solution from the oxidation and utilized.

A cheap and particularly suitable nitrate solution for the present purposes is found in the waste liquor from the manufacture of lead chromate; a liquid which is ordinarily sent to the sewer and which is hereinafter termed "chromate waste liquor." Lead chromate is ordinarily made by double decomposition between a solution of lead nitrate and a solution of an alkali bichromate or chromate. Ordinarily sodium bichromate or chromate is employed; more rarely, the potassium salt is used. Chromate of lead is formed and precipitated by a well-known reaction and nitric acid and alkali nitrate remain in the solution. With a bichromate, half the nitric acid is free and half is in a combined form. Where sodium bichromate and lead nitrate are used as is usually the case, for each molecule of lead chromate formed there remains in the residual solution a molecule of sodium nitrate and a molecule of free nitric acid. This residual solution, or chromate waste liquor, I find particularly suitable for my purposes since it exercises a very vigorous action upon finely divided lead in the presence of air and forms a desirable type of hydrated or basic reactive lead oxid. While solutions for my purpose may be formed by direct solution of commercial nitrate of soda in water, I prefer this chromate waste liquor not only on account of its cheapness but because of its advantages in practical work. It seems to be rather more reactive than a directly produced nitrate solution.

The free nitric acid in the waste liquor may be preliminarily neutralized by soda or soda ash to convert it into sodium nitrate; but this is not ordinarily necessary. If not so neutralized however it undergoes far-reaching reduction in the process, even so far as ammonia, and is, or may be, ultimately not recovered as a useful product as is the case where it is converted into sodium nitrate which may be recovered later as sodium nitrite. The presence of free nitric acid in the liquor to begin with is however often advantageous in my process for the reason that with some varieties of comminuted lead carrying oxidized coating layers it exercises a solvent action on the oxid in the beginning of the operation upon

a charge of lead, much accelerating the progress of the oxidizing action.

Any of the ordinary finely divided forms of lead, such as moss lead, dust lead, blue lead and the like, may be employed. Blue fume is not so suitable since it contains lead sulfate and sulfid. Lead shavings and chips are likewise not so well adapted being too coarse. In the present process, the lead should be in a state of quite fine subdivision. Any apparatus adapted to give a good aeration of lead in the presence of liquid may be employed in my process, such as rotating drums and the other apparatus often employed for oxidizing lead by wet processes. It is not necessary to use high heats or any heat beyond atmospheric and it is also unnecessary to use artificial cooling. Whatever the form of apparatus employed, it should be such as to give efficient aeration since in the present process the oxygen of the air is relied upon for the major part of the oxidation, the nitrate acting largely as a facilitating reagent.

Any strength of nitrate solution between two per cent. and 50 per cent. may be employed. A solution containing as little as two per cent. is efficient as a catalyzing agent; but with stronger solutions where the sodium nitrite is to be subsequently recovered the operation is cheaper as involving less expense in such recovery. The relative amount of liquid may vary from enough to cover the lead and form a body of liquid to merely enough to convert the lead into a sloppy mass.

The possibility of the cheap production of nitrite is one of the valuable features of the present invention, and where such recovery is effected of course the use of strong solutions of nitrate producing final strong solutions of nitrite is desirable. While potassium nitrate, or waste chromate liquor containing potassium nitrate, may be employed in this invention it offers no advantage over sodium nitrate, or waste chromate liquor containing sodium nitrate; and I regard sodium nitrate, for many reasons, as in any event being rather better adapted for my purposes.

In a practical embodiment of the described process, I may place 4000 pounds of dust lead in a drum with 400 gallons of waste chromate liquor, containing, say, 8 per cent. of sodium nitrate and 4 per cent. of free nitric acid and agitate with free access of air for 24 to 48 hours. The lead is thereby converted into a reddish orange hydrated reactive basic oxid of large bulk for its weight while the nitric acid of the original solution disappears and the sodium nitrate is converted into an equivalent amount of sodium nitrite. The oxid may be separated from the residual liquid by any convenient means, such as subsidence

and pressing and washing, and may be marketed as it is, or, and usefully, it may be converted into pigmentary products for which its state of subdivision and molecular constitution render it particularly well adapted. By a gentle heating it may be dehydrated and converted into massicot of exceptional quality, while a continuation of the heating under oxidizing conditions converts it into an extremely high grade red lead. By modifying the heating conditions it may, of course, be converted into a very fine-grained litharge. The hydrated oxid may be gassed with carbon dioxide to convert it into white lead. The chromate waste liquor may, or may not, be neutralized with sodium carbonate or bicarbonate preliminarily. If so neutralized the quantity of sodium nitrite to be recovered is increased and some advantages are gained in the operation. The liquor from which the hydrated oxid is separated may be simply evaporated to regain sodium nitrite.

The preliminary separation of the residual liquor may be omitted where red lead is to be made, the material being dried and furnace-dried to produce red lead. The presence of the nitrite facilitates the oxidation to red lead and after the red lead is formed, the nitrite may then be leached out and regained. In this modification of my invention, in the finishing stages of the first or aerial oxidation the water of the solution may be allowed to evaporate and pass away with the air to a large extent as reducing the cost of the subsequent drying prior to the red lead oxidation.

Where the nitrite solution is separated from the hydrated oxid preliminarily to drying and re-oxidation to red lead, if the hydrated oxid be not washed too thoroughly enough nitrite will remain in it to aid materially in such reoxidation. While alkali nitrites do not appear to be changed or destroyed to any extent in the oxidation of lead protoxid to minium or red lead their presence gives a smoother and quicker oxidation with the production of a better article. With small amounts of nitrite, say from one per cent. down, it need not be removed from the finished red lead. A quarter per cent. of nitrite is sufficient to aid materially in making red lead.

In a typical embodiment of my process in making red lead, finely divided lead may be oxidized by air in the presence of sodium nitrate solution, or "waste chromate liquor" in the manner previously described and after completion of the reaction the lead oxid may be separated from the bulk of the solution

by subsidence and draining and then dried without washing. The dried material may then be furnace-dried under oxidizing conditions at a low temperature to convert it into red lead and then directly marketed without leaching.

I claim:

1. The process of oxidizing lead which comprises exposing finely divided lead to the simultaneous action of a solution of an alkali nitrate and of air. 70

2. The process of oxidizing lead which comprises exposing finely divided lead to the simultaneous action of a solution of an alkali nitrate and of air, to obtain a mass comprising oxidized lead and alkali nitrite. 75

3. The process of oxidizing lead which comprises exposing finely divided lead to the simultaneous action of a solution of sodium nitrate and of air. 80

4. The process of oxidizing lead which comprises exposing finely divided lead to the simultaneous action of chromate waste liquor containing alkali nitrate and of air. 85

5. The process of oxidizing lead which comprises exposing finely divided lead to the simultaneous action of chromate waste liquor containing sodium nitrate and of air, and thereafter separating oxidized lead and sodium nitrite. 90

6. The process of oxidizing lead which comprises exposing finely divided lead to the simultaneous action of neutralized chromate waste liquor containing alkali nitrate and of air. 95

7. The process of oxidizing lead which comprises exposing finely divided lead to the simultaneous action of neutralized chromate waste liquor containing sodium nitrate and of air, and thereafter separating sodium nitrite and oxidized lead. 100

8. The process of making lead oxid which comprises exposing finely divided lead to the simultaneous action of air and alkali nitrate solution, recovering the lead oxid, and then converting such oxid into red lead by heat and oxidation. 105

9. The process of making lead oxid which comprises exposing finely divided lead to the simultaneous action of air and sodium nitrate solution, recovering the lead oxid, and then converting such oxid into red lead by heat and oxidation. 110

In testimony whereof, I affix my signature in the presence of witnesses.

CLIFFORD D. HOLLEY.

Witnesses:

N. J. SEPIN,  
H. E. CLARK.